



US010233521B2

(12) **United States Patent**  
**Stewart**

(10) **Patent No.:** **US 10,233,521 B2**  
(b4) **Date of Patent:** **Mar. 19, 2019**

(54) **LOW COBALT HARD FACING ALLOY**(71) Applicant: **ROLLS-ROYCE plc**, London (GB)(72) Inventor: **David A Stewart**, Derby (GB)(73) Assignee: **ROLLS-ROYCE plc**, London (GB)

(\*) Notice: Subject to any disclaimer, the term of this patent is extended or adjusted under 35 U.S.C. 154(b) by 110 days.

(21) Appl. No.: **15/402,821**(22) Filed: **Jan. 10, 2017**(65) **Prior Publication Data**

US 2017/0218490 A1 Aug. 3, 2017

(30) **Foreign Application Priority Data**

Feb. 1, 2016 (GB) ..... 1601765.9

(51) **Int. Cl.****C22C 38/00** (2006.01)**C22C 38/04** (2006.01)**C22C 38/34** (2006.01)**C22C 38/48** (2006.01)**C22C 38/50** (2006.01)**C22C 38/52** (2006.01)(52) **U.S. Cl.**CPC ..... **C22C 38/52** (2013.01); **C22C 38/001** (2013.01); **C22C 38/002** (2013.01); **C22C 38/04** (2013.01); **C22C 38/34** (2013.01); **C22C 38/48** (2013.01); **C22C 38/50** (2013.01)(58) **Field of Classification Search**

CPC ..... C22C 38/001; C22C 38/002; C22C 38/04; C22C 38/34; C22C 38/48; C22C 38/50; C22C 38/52

See application file for complete search history.

(56) **References Cited**

## U.S. PATENT DOCUMENTS

- 4,077,801 A \* 3/1978 Heyer ..... C22C 19/055  
148/427  
4,812,177 A \* 3/1989 Maehara ..... C21D 8/005  
148/505  
4,854,185 A \* 8/1989 Lichtenberg ..... F16C 1/226  
188/196 B  
4,981,647 A \* 1/1991 Rothman ..... C22C 30/00  
420/43  
5,296,054 A \* 3/1994 Lvovich et al.  
5,310,431 A \* 5/1994 Buck ..... C22C 38/52  
148/325  
5,512,237 A \* 4/1996 Stigenberg ..... C22C 38/42  
420/38

- 5,514,328 A \* 5/1996 Menon ..... C22C 38/52  
420/36  
5,660,939 A 8/1997 Burdett ..... C22C 30/00  
148/442  
5,820,817 A \* 10/1998 Angeliu ..... C22C 38/002  
420/40  
5,944,922 A \* 8/1999 Kadoya ..... C21D 6/004  
148/325  
RE36,382 E \* 11/1999 Hultin-Stigenberg ..... C22C 38/42  
420/38  
6,165,627 A \* 12/2000 Miyazaki ..... C22C 38/105  
148/320  
6,174,385 B1 \* 1/2001 Morinaga ..... C22C 38/00  
148/325  
6,426,038 B1 \* 7/2002 Fedchun ..... C22C 38/002  
420/104  
6,426,040 B1 \* 7/2002 Fedchun ..... C22C 38/002  
420/104  
6,464,804 B2 \* 10/2002 Goecmen ..... C21D 6/004  
148/325  
6,479,013 B1 \* 11/2002 Sera ..... B22D 17/2023  
148/325  
6,485,679 B1 \* 11/2002 Sundstrom ..... C22C 38/44  
420/38  
6,630,103 B2 \* 10/2003 Martin ..... C21D 6/02  
148/325  
6,667,005 B2 \* 12/2003 Ishida ..... C22C 38/42  
148/333  
6,685,881 B2 \* 2/2004 Hamano ..... C22C 38/001  
420/41  
6,702,905 B1 \* 3/2004 Qiao ..... C21D 6/002  
148/326  
6,764,645 B2 \* 7/2004 Hayaishi ..... C22C 38/001  
148/622

(Continued)

## FOREIGN PATENT DOCUMENTS

- EP 0 265 165 A2 4/1988  
EP 0 735 155 A1 10/1996

(Continued)

## OTHER PUBLICATIONS

Aug. 1, 2017 Extended Search Report issued in European Patent Application No. 17150539.9.

Aug. 2, 2016 Search Report issued in British Patent Application No. 1601765.9.

\* cited by examiner

Primary Examiner — Cam N. Nguyen

(74) Attorney, Agent, or Firm — Oliff PLC

(57) **ABSTRACT**

A stainless steel alloy including essentially of 19 to 22 percent by weight chromium, 8.5 to 10.5 percent by weight nickel, 5.25 to 5.75 percent by weight silicon, 0.25 to 1.2 percent by weight carbon, 4.0 to 6.0 percent by weight niobium, 0.3 to 0.5 percent by weight titanium and the balance iron plus impurities. The impurities may include 0 to 0.2 percent by weight cobalt, 0 to 0.5 percent by weight manganese, 0 to 0.3 percent by weight molybdenum, 0 to 0.03 percent by weight phosphor, 0 to 0.03 percent by weight sulphur, 0 to 0.1 percent by weight nitrogen.

12 Claims, No Drawings

(56)

## References Cited

## U.S. PATENT DOCUMENTS

- |           |      |         |                 |                           |
|-----------|------|---------|-----------------|---------------------------|
| 6,769,414 | B2 * | 8/2004  | Rembold .....   | F02D 33/006<br>123/179.17 |
| 6,773,519 | B2 * | 8/2004  | Fujita .....    | C21D 9/38<br>148/335      |
| 6,773,661 | B2 * | 8/2004  | Hayaishi .....  | C22C 38/14<br>420/84      |
| 6,793,745 | B2 * | 9/2004  | Weber .....     | C21D 6/004<br>148/325     |
| 6,818,072 | B2 * | 11/2004 | Kondo .....     | C21D 8/10<br>148/320      |
| 6,866,816 | B2 * | 3/2005  | Liang .....     | C22C 33/0285<br>148/324   |
| 6,890,393 | B2 * | 5/2005  | Buck .....      | C21D 6/004<br>148/325     |
| 6,896,747 | B2 * | 5/2005  | Hauser .....    | C21D 8/065<br>148/327     |
| 6,899,773 | B2 * | 5/2005  | Buck .....      | C21D 6/004<br>148/325     |
| 7,153,373 | B2 * | 12/2006 | Maziasz .....   | C21D 6/005<br>148/327     |
| 7,160,399 | B2 * | 1/2007  | Kuehmann .....  | C21D 6/02<br>148/326      |
| 7,235,212 | B2 * | 6/2007  | Kuehmann .....  | C21D 6/02<br>420/107      |
| 7,255,755 | B2 * | 8/2007  | Maziasz .....   | C21D 6/005<br>148/327     |
| 7,258,752 | B2 * | 8/2007  | Maziasz .....   | C22C 38/001<br>148/326    |
| 7,297,214 | B2 * | 11/2007 | Ishida .....    | C22C 19/055<br>148/310    |
| 7,326,307 | B2 * | 2/2008  | Ueta .....      | C22C 38/02<br>148/327     |
| 7,425,240 | B2 * | 9/2008  | Guelton .....   | C21D 8/0415<br>148/541    |
| 7,611,590 | B2 * | 11/2009 | Liang .....     | B22F 5/008<br>148/324     |
| 7,651,575 | B2 * | 1/2010  | Sawford .....   | C22C 19/058<br>148/410    |
| 7,658,883 | B2 * | 2/2010  | Marya .....     | C22C 38/001<br>148/327    |
| 7,686,898 | B2 * | 3/2010  | Nazmy .....     | C22C 38/001<br>148/325    |
| 7,700,037 | B2 * | 4/2010  | Westin .....    | C22C 38/001<br>420/128    |
| 7,708,841 | B2 * | 5/2010  | Saller .....    | C22C 38/58<br>148/327     |
| 7,718,014 | B2 * | 5/2010  | Usami .....     | B23K 35/3053<br>148/332   |
| 7,731,896 | B2 * | 6/2010  | Usami .....     | B23K 35/3053<br>420/119   |
| 7,744,813 | B2 * | 6/2010  | Brady .....     | C22C 38/02<br>148/326     |
| RE41,504  | E *  | 8/2010  | Maziasz .....   | C21D 6/005<br>148/327     |
| 7,922,968 | B2 * | 4/2011  | Son .....       | C22C 38/02<br>148/320     |
| 8,012,269 | B2 * | 9/2011  | Yamamoto .....  | C22C 38/002<br>148/101    |
| 8,025,839 | B2 * | 9/2011  | Jonson .....    | C22C 38/24<br>148/325     |
| 8,192,682 | B2 * | 6/2012  | Maziasz .....   | E21B 36/04<br>148/326     |
| 8,313,589 | B2 * | 11/2012 | Takasawa .....  | C21D 1/28<br>148/330      |
| 8,317,944 | B1 * | 11/2012 | Jablonski ..... | C23C 12/02<br>148/325     |
| 8,317,946 | B2 * | 11/2012 | Arai .....      | C21D 8/10<br>148/335      |

- |           |      |         |                        |                         |
|-----------|------|---------|------------------------|-------------------------|
| 8,318,083 | B2 * | 11/2012 | Pankiw .....           | C22C 30/00<br>148/327   |
| 8,337,748 | B2 * | 12/2012 | Rakowski .....         | C22C 38/38<br>148/325   |
| 8,337,749 | B2 * | 12/2012 | Bergstrom .....        | C22C 38/42<br>420/56    |
| 8,414,715 | B2 * | 4/2013  | Altschuler .....       | C21D 1/25<br>148/590    |
| 8,430,075 | B2 * | 4/2013  | Qiao .....             | C22C 38/02<br>123/188.3 |
| 8,431,072 | B2 * | 4/2013  | Muralidharan .....     | B22D 25/06<br>420/43    |
| 8,444,776 | B1 * | 5/2013  | Bailey .....           | C21D 6/001<br>148/335   |
| 8,454,765 | B2 * | 6/2013  | Saller .....           | C22C 38/58<br>148/327   |
| 8,460,800 | B2 * | 6/2013  | Hoshika .....          | C22C 38/001<br>428/213  |
| 8,479,700 | B2 * | 7/2013  | Qiao .....             | C22C 1/02<br>123/188.3  |
| 8,540,933 | B2 * | 9/2013  | Nylof .....            | C22C 38/001<br>148/325  |
| 8,562,761 | B2 * | 10/2013 | Gunnarsson .....       | C21D 1/25<br>148/328    |
| 8,580,050 | B2 * | 11/2013 | Morita .....           | C22C 38/001<br>148/316  |
| 8,580,190 | B2 * | 11/2013 | Hattendorf .....       | C22C 38/001<br>148/325  |
| 8,623,108 | B2 * | 1/2014  | Theisen .....          | B22F 9/082<br>420/127   |
| 8,784,278 | B2 * | 7/2014  | Flake .....            | A63B 22/0264<br>482/54  |
| 9,051,634 | B2 * | 6/2015  | Morohoshi .....        | C21D 9/46               |
| 9,121,088 | B2 * | 9/2015  | Bailey .....           | C21D 1/56               |
| 9,121,089 | B2 * | 9/2015  | Bergstrom .....        | C22C 38/42              |
| 9,133,538 | B2 * | 9/2015  | Rakowski .....         | C22C 38/38              |
| 9,157,131 | B2 * | 10/2015 | Zou .....              | C21D 1/667              |
| 9,181,597 | B1 * | 11/2015 | Hawk .....             | C21D 6/002              |
| 9,200,343 | B2 * | 12/2015 | Matsuda .....          | C21D 9/46               |
| 9,228,250 | B2 * | 1/2016  | Alves .....            | B23K 35/0261            |
| 9,284,631 | B2 * | 3/2016  | Radon .....            | C22C 37/10              |
| 9,334,547 | B2 * | 5/2016  | Qiao .....             | C21D 9/0068             |
| 9,347,121 | B2 * | 5/2016  | Forbes Jones .....     | C22C 38/42              |
| 9,458,743 | B2 * | 10/2016 | Qiao .....             | C21D 5/00               |
| 9,499,890 | B1 * | 11/2016 | Zhang .....            | C22C 38/50              |
| 9,513,071 | B2 * | 12/2016 | Sjodin .....           | B23K 35/308             |
| 9,513,072 | B2 * | 12/2016 | Sjodin .....           | B23K 35/308             |
| 9,555,158 | B2 * | 1/2017  | Meyer-Kobbe .....      | C21D 6/002              |
| 9,556,503 | B1 * | 1/2017  | Hawk .....             | C22C 38/54              |
| 9,593,916 | B2 * | 3/2017  | Bailey .....           | C21D 6/001              |
| 9,657,382 | B2 * | 5/2017  | Funakawa .....         | C22C 38/001             |
| 9,689,050 | B2 * | 6/2017  | Bouaziz .....          | C21D 6/02               |
| 9,689,061 | B2 * | 6/2017  | Angles .....           | C22C 38/12              |
| 9,702,641 | B2 * | 7/2017  | Sjodin .....           | B23K 35/308             |
| 9,797,033 | B2 * | 10/2017 | Li .....               | C22C 38/38              |
| 9,803,267 | B2 * | 10/2017 | Roscoe .....           | C22C 38/34              |
| 9,816,165 | B2 * | 11/2017 | Li .....               | C22C 38/32              |
| 9,822,435 | B2 * | 11/2017 | Bergstrom .....        | C22C 38/42              |
| 9,845,518 | B2 * | 12/2017 | Cobo .....             | C21D 9/0068             |
| 9,869,009 | B2 * | 1/2018  | Vartanov .....         | C21D 9/30               |
| 9,873,932 | B2 * | 1/2018  | Bergstrom .....        | C22C 38/58              |
| 9,903,023 | B2 * | 2/2018  | Maruyama .....         | C23C 30/005             |
| 9,919,385 | B2 * | 3/2018  | Sjodin .....           | B23K 35/308             |
| 9,932,867 | B2 * | 4/2018  | Qiao .....             | F01L 3/02               |
| 9,963,766 | B2 * | 5/2018  | Sachadel-Solarek ..... | C22C 38/54              |
| 9,981,346 | B2 * | 5/2018  | Han, II .....          | B23K 35/0266            |

#### FOREIGN PATENT DOCUMENTS

GE  
IP

2 167 088 A 5/1986  
H06-170584 A 6/1994

## 1

## LOW COBALT HARD FACING ALLOY

## FIELD OF THE INVENTION

The present invention relates to steel alloys and particularly a chromium nickel silicon stainless steel alloy with low cobalt that may be suited for use in nuclear reactors, particularly in the components used in the steam generating plant of nuclear reactors.

## BACKGROUND OF THE INVENTION

Traditionally, cobalt-based alloys, including Stellite® alloys, have been used for wear-based applications including, for example, in nuclear power applications. The alloys may be used to both form components or to provide hard-facing where harder or tougher material is applied to a base metal or substrate.

It is common for hard-facing to be applied to a new part during production to increase its wear resistance. Alternatively, hard-facing may be used to restore a worn surface. Extensive work in research has resulted in the development of a wide range of alloys and manufacturing procedures dependent on the properties and/or characteristics of the required alloy.

Within the nuclear industry the presence of cobalt within an alloy gives rise to the potential for the cobalt to activate within a neutron flux to result in the radioisotope cobalt-60 which has a long half-life. This makes the use of cobalt undesirable for alloys used in this industry. The cobalt may be released as the alloy wears through various processes, one of which is galling that is caused by adhesion between sliding surfaces caused by a combination of friction and adhesion between the surfaces, followed by slipping and tearing of crystal structure beneath the surface. This will generally leave some material stuck or even friction welded to the adjacent surface, whereas the galled material may appear gouged with balled-up or torn lumps of material stuck to its surface.

Replacements for Stellite have been developed by the industry with low or nil cobalt quantities. Exemplary alloys are detailed in the table below:

| Alloy                   | Cr    | C       | Nb      | Nb + Va | Ni       | Si        | Fe  | Co  | Ti      |
|-------------------------|-------|---------|---------|---------|----------|-----------|-----|-----|---------|
| GB2167088               | 15-25 | 1-3     |         | 5-15    | 5-15     | 2.7-5.6   | Bal | Nil | Nil     |
| T5183                   | 19-22 | 1.8-2.2 | 6.5-8.0 |         | 8.5-10.5 | 4.5-5.25  | Bal | 0.2 | Trace   |
| U.S. Pat. No. 5,660,939 | 19-22 | 1.7-2.0 | 8.0-9.0 |         | 8.5-10.5 | 5.25-5.75 | Bal | 0.2 | 0.3-0.7 |

In GB2167088 niobium is provided, but always with the presence of vanadium, which prevents the chromium from combining with the carbon and weakening the matrix. The vanadium also acts as a grain refiner within the wholly austenitic alloy that helps the keep the size of the grains within the alloy within an acceptable range.

The alloys of U.S. Pat. No. 5,660,939 modified the alloy of T5183 by the deliberate addition of titanium and by increasing the amounts of niobium and silicon. The controlled additions of titanium, niobium and silicon alter the structure of the steel to provide a duplex austenitic/ferritic microstructure which undergoes secondary hardening due to the formation of an iron silicon intermetallic phase.

Further hardening is achievable by hot isostatic pressing (HIPPING) of the stainless steel alloy when in powder form where secondary hardening occurs within the ferritic phase of the duplex microstructure.

## 2

The niobium provides a preferential carbide former over chromium, enabling high chromium levels to be maintained within the matrix so as to give good corrosion performance. Low cobalt based alloys, or cobalt alloy replacements, typically comprise significant quantities of carbide forming elements which can form alloys with hardness values in excess of 500 Hv. As with traditional Stellite alloys, the high levels of hardness observed can make machining difficult, resulting in poor mechanical properties for, for example, ductility, fracture toughness, impact resistance and workability. Additionally, the cost of using such alloys is high due to the need for special treatments and/or precision casting or other near net shape manufacturing methods to limit further machining.

Accordingly, it would therefore be advantageous to provide an alloy without the aforementioned disadvantages.

## SUMMARY OF THE INVENTION

The present invention accordingly provides, in a first aspect, an alloy consisting essentially of 19 to 22 percent by weight chromium, 8.5 to 10.5 percent by weight nickel, 5.25 to 5.75 percent by weight silicon, 0.25 to 1.2 percent by weight carbon, 4.0 to 6.0 percent by weight niobium, 0.3 to 0.5 percent by weight titanium, 0.1 to 0.5 percent by weight nitrogen and the balance iron plus impurities.

The impurities may consist of 0 to 0.2 percent by weight cobalt, 0 to 0.5 percent by weight manganese, 0 to 0.3 percent by weight molybdenum, 0 to 0.03 percent by weight phosphorus, 0 to 0.03 percent by weight sulphur.

The alloy may comprise 0.8 to 1.2 percent by weight carbon.

The alloy may be in powder form which is consolidated in a hot isostatic press.

The alloy may be applied to an article to provide a coating on the article. The coating may be hard faced or welded onto the article.

The alloy may be used in a steam generating plant. The steam may be generated through a nuclear reaction.

An alloy consisting essentially of 19 to 22 percent by weight chromium, 8.5 to 10.5 percent by weight nickel, 5.25 to 5.75 percent by weight silicon, 0.25 to 1.2 percent by

weight carbon, 4.0 to 6.0 percent by weight niobium, 0.3 to 0.5 percent by weight titanium, 0 to 0.2 percent by weight cobalt, 0 to 0.5 percent by weight manganese, 0 to 0.3 percent by weight molybdenum, 0 to 0.03 percent by weight phosphorus, 0 to 0.03 percent by weight sulphur, 0 to 0.5 percent by weight nitrogen and the balance iron plus impurities.

A preferred embodiment of the present invention will now be described, by way of example only.

## DETAILED DESCRIPTION OF THE PREFERRED EMBODIMENTS

The improved alloys described here have been developed having, in weight percent, 19 to 22 chromium, 8.5 to 10.5 nickel, 5.25 to 5.75 silicon, 4.0 to 6.0 niobium, 0.3 to 0.5

titanium, 0.25 to 1.2 carbon, 0.1 to 0.5 percent by weight nitrogen and the balance iron plus incidental impurities. The alloy may have carbon in the range 0.8 to 1.2 wt %.

The impurities may be up to 0.2 wt % cobalt, up to 0.5 wt % manganese, up to 0.3 wt % molybdenum, up to 0.03 wt % phosphor, up to 0.03 wt % sulphur.

These compositions are similar to those proposed in U.S. Pat. No. 5,660,939 but the reduction in the carbon and niobium content has been found to improve the ductility of the alloy. The nitrogen has been found to aid the galling resistance of the matrix.

The new alloy has an acceptable galling resistance as carbides will still be formed, and the matrix continues to have a duplex austenitic/ferritic microstructure which undergoes secondary hardening due to the formation of an iron silicon intermetallic phase.

Although carbides continue to be formed the alloy has a resultant lower overall carbide caused, in part, by the weight percentage content of niobium and carbon that give an alloy with an acceptable hardness but greater ductility and toughness. This improvement in ductility opens up the range of range of applications where consideration to shock events has to be considered as well as the overall wear resistance requirement.

The invention claimed is:

1. An alloy consisting essentially of 19 to 22 percent by weight chromium, 8.5 to 10.5 percent by weight nickel, 5.25 to 5.75 percent by weight silicon, 0.25 to 1.2 percent by weight carbon, 4.0 to 6.0 percent by weight niobium, 0.3 to 0.5 percent by weight titanium, 0.1 to 0.5 percent by weight nitrogen and the balance iron plus impurities.

2. An alloy according to claim 1 wherein the impurities consist of 0 to 0.2 percent by weight cobalt, 0 to 0.5 percent by weight manganese, 0 to 0.3 percent by weight molybdenum, 0 to 0.03 percent by weight phosphor, 0 to 0.03 percent by weight sulphur.

3. An article comprising an alloy as claimed in claim 2.

4. An article having a coating comprising an alloy as claimed in claim 2.

5. An alloy according to claim 1, wherein the alloy comprises 0.8 to 1.2 percent by weight carbon.

6. An article comprising an alloy as claimed in claim 5.

7. An article having a coating comprising an alloy as claimed in claim 5.

8. An article comprising an alloy as claimed in claim 1.

9. An article having a coating comprising an alloy as claimed in claim 1.

10. An alloy consisting essentially of 19 to 22 percent by weight chromium, 8.5 to 10.5 percent by weight nickel, 5.25 to 5.75 percent by weight silicon, 0.25 to 1.2 percent by weight carbon, 4.0 to 6.0 percent by weight niobium, 0.3 to 0.5 percent by weight titanium, 0 to 0.2 percent by weight cobalt, 0 to 0.5 percent by weight manganese, 0 to 0.3 percent by weight molybdenum, 0 to 0.03 percent by weight phosphor, 0 to 0.03 percent by weight sulphur, 0 to 0.5 percent by weight nitrogen and the balance iron plus impurities.

11. An alloy according to claim 10 wherein the alloy comprises 0.8 to 1.2 percent by weight carbon.

12. An article comprising an alloy as claimed in claim 10.

\* \* \* \* \*